

## UNITED STATES PATENT OFFICE

2,426,861

## PROCESS FOR IMPROVING THE PROPERTIES OF WATER-INSOLUBLE ARTIFICIAL PROTEIN FIBRES

Giampiero Comolli, Milan, Italy, assignor to  
Sandoz A. G., Basel, SwitzerlandNo Drawing. Application November 6, 1939.  
Serial No. 303,158. In Italy November 14, 1938

5 Claims. (Cl. 8—127.6)

1

The present invention relates to the treatment of insoluble artificial fibres manufactured from solutions of substances of a protein-like nature, such as casein, keratin and the like, for the purpose of increasing their resistance to physical and chemical agents without impairing their tintorial properties.

According to the present invention it has been found that if an insoluble artificial fibre manufactured from a solution of a proteinic substance, for instance artificial fibre prepared from casein, is subjected to a treatment with chromium compounds, there is a very appreciable improvement in the dynamometric resistance of the fibre itself (in the moist as well as in the dry state), in the resistance to fulling, friction and wear, in the resistance to the action of boiling water even in the presence of acid or alkali and also in the resistance to the action of hot iron (ironing), and there is also an increase in the fastness of the dyeings produced thereon with acid dyestuffs and chrome dyestuffs as well as with direct dyestuffs and dyestuffs belonging to other categories.

The artificial fibre, when subjected to the treatment hereinafter described, undergoes an action similar to the action produced on depilated skins when subjected to chrome tanning with one or two immersions, which acquire great tenacity and powerful resistance to stretching and are not affected by boiling water.

This treatment enables, furthermore, the above-mentioned artificial fibres to absorb and retain dyestuffs in a much higher condition of stability than is the case with artificial fibres obtained from protein-like material not subjected to the process which forms the subject matter of the patent. In fact, acid dyestuffs which when applied on untreated fibres do not resist even light washing, on the contrary after treatment according to the present invention they withstand very well washing at 60° C. in presence of soap and carbonate of soda. Moreover, the treatment in question makes it possible to dye with all chrome dyestuffs generally without impairing the resistance of the artificial fibre, contrary to what happens in the case of dyed fibres obtained from protein-like substances and not treated by the process which forms the subject matter of this invention.

The treatment which is covered by this invention and can be used in the actual manufacture of artificial fibres formed of or containing protein-like substances, is based on the use of salts of chromium (chrome alum, chromium sulphate,

2

chromium chloride, etc., either normal or of various degrees of basicity). If desired the treatment may be effected with two baths, the first containing for example sodium or potassium bichromate and the other containing products capable of converting the compounds of chromic anhydride into compounds of chromium sesquioxide.

In the preparation of this second bath the following compounds can be used:

(a) Sodium thiosulphate, sodium bisulphite, sulphurous acid and its derivatives or any other reducing means or substance.

(b) Any oxidising means or substance capable of converting chromic acid into perchromic acid which, owing to its instability, can produce compounds of chromium sesquioxide.

The following examples illustrate how the invention may be carried out in practice, but it is to be understood that the invention is in no way limited by the details given in these examples.

## Example 1

Artificial fibre prepared from casein is impregnated in a bath containing 100 grams per litre of potassium bichromate with the addition, if desired, of a mineral acid. After the impregnation of the fibre it is squeezed and placed in another bath containing 100 grams per litre of sodium bisulphite and then thoroughly washed with water. The fibre so treated acquires all the properties above mentioned (better resistance to stretching, wear, boiling water, etc.).

## Example 2

The artificial fibre treated as described in Example 1 is dyed with acid dyestuffs. A comparative examination shows that the dyes obtained on the fibre treated by the process above described present a very high fastness to washing, which is equal to that on wool, whilst the fastness of the dyes on material untreated is practically nil.

## Example 3

Artificial fibre treated as in Example 1 is dyed with chrome dyes by the afterchroming process as well as in the dyeing process with a single bath.

The alkaline fulling of the dyed material does not exercise any negative influence upon the shade and the resistance of the fibres, whilst similar dyeings executed on untreated fibre are practically unusable after having been subjected to alkaline fulling.

## Example 4

Artificial casein fibre is soaked in a 10% aqueous sodium bichromate solution at 35° C. until the material is uniformly impregnated, hydro-extracted and the yellow colored wet fibre introduced into a 10% aqueous solution of sodium bisulphite, whereby the color of the fibre rapidly becomes green. When the reduction of the chromic acid is finished, the material is rinsed and dried. It possesses the same properties as the material treated according to Example 1. Instead of sodium bichromate one can use the respective potassium salt, and instead of sodium bisulphite, the sodium hydrosulphite, thiosulphate or gaseous sulphurous acid mixed with steam.

## Example 5

100 parts of casin staple fibres are treated in a milling drum during 10 minutes with a 30-40° C. warm solution of 8-10 parts of sodium- or potassium bichromate in 400-500 parts of water. Thereon 4 parts of hydrochloric acid or a corresponding quantity of sulphuric acid are added thereto in order to liberate the chromic acid. After 20 minutes the major part of the chromic acid has been taken up by the fibre and the solution is coloured only weakly yellow. For the reduction, there is added a solution of 12-15 parts of sodium bisulphite and the drum allowed to run until the green solution becomes almost colorless. The fibres are then rinsed, treated with some ammonia or another alkali like soda, etc., in order to neutralize the free acid, and carefully washed out.

## Example 6

A mixed textile material consisting of 50 parts of casein fibre and of 50 parts of vegetable, rayon or animal fibres is treated in the manner described in the previous examples and the treated material carefully washed and neutralized after the tanning.

The textile material subjected to such treatment can then be dyed with any desired dye-stuffs. Acid and chrome dyestuffs dye casein and animal fibres, whereas substantive dyestuffs dye casein and cellulosic fibres; therefore, any desired combination of shade may be produced.

The textile material treated and dyed according to the example possesses a much better touch and better dynamometric properties as compared with the material that has not been subjected to the tanning operation.

## Example 7

100 parts of casein yarn are treated during 18 hours at 25° C. in a solution of the following composition:

|                            | Parts |
|----------------------------|-------|
| Water                      | 1000  |
| Chrome alum                | 120   |
| Anhydrous sodium carbonate | 12    |

and if necessary 3 parts of a wetting agent which is resistant to chrome salts.

After this treatment the yarn is hydroextracted, washed out, treated during 2 minutes in 1000 parts of water containing 2 parts of concentrated ammonia, washed again, hydroextracted and dried.

The casein fibre which is colored in a clear olive green shade possesses a smooth touch which remains, even after a subsequent dyeing in a bath containing mineral acid. The resistance to breaking and the elasticity of the casein fibre treated in this manner is much better as compared with

70  
75

the casein fibre which has not been subjected to the above treatment.

What I claim is:

1. A process for producing water-insoluble artificial casein fiber, which comprises the steps of impregnating hardened fiber, prepared from a casein solution by a spinning and hardening process, with a solution of a water-soluble chromium compound, and then converting the latter into a water-insoluble chromium compound by treatment of the impregnated fiber with a reducing agent, thereby causing the formation and fixation of the water-insoluble chromium compound in and on the treated fiber.
2. A process for producing water-insoluble artificial casein fiber, which comprises the steps of impregnating hardened fiber, prepared from a casein solution by a spinning and hardening process, with a solution of a water-soluble salt of chromic acid, and then converting the latter into a water-insoluble chromium compound by treatment of the impregnated fiber with a reducing agent, thereby causing the formation and fixation of the water-insoluble chromium compound in and on the treated fiber.
3. A process for producing water-insoluble artificial casein fiber, which comprises the steps of impregnating hardened fiber, prepared from a casein solution by a spinning and hardening process, with a solution of a water-soluble salt of chromic acid, and then treating the impregnated fiber with a solution of a reducing agent.
4. A process for producing water-insoluble artificial casein fiber, which comprises the steps of impregnating hardened fiber, prepared from a casein solution by a spinning and hardening process, with a solution of an alkali metal bichromate, and then treating the impregnated fiber with a solution of an alkali metal bisulphite.
5. Water-insoluble artificial casein fiber comprising an insolubilized fiber body prepared from a casein solution by a spinning and hardening process, and containing a subsequently-incorporated water-insoluble chromium compound in and on said fiber body, said fiber possessing improved dynamometric resistance and improved fastness to boiling water, milling, washing and dyeing, as compared with the same insolubilized artificial fiber free from said water-insoluble chromium compound.

GIAMPIERO COMOLLI.

## REFERENCES CITED

55 The following references are of record in the file of this patent:

## UNITED STATES PATENTS

| Number    | Name              | Date          |
|-----------|-------------------|---------------|
| 77,990    | Lowrey            | May 19, 1868  |
| 625,345   | Millar            | Oct. 15, 1898 |
| 836,788   | Todtenhaupt       | Nov. 27, 1906 |
| 950,435   | Chavassieu        | Feb. 22, 1910 |
| 1,865,497 | Atwood            | July 5, 1932  |
| 2,103,163 | Lange             | Dec. 21, 1937 |
| 2,120,851 | Becker et al.     | June 14, 1938 |
| 2,140,274 | Whittier et al.   | Dec. 13, 1938 |
| 2,169,955 | Oosterbeek et al. | Aug. 15, 1939 |
| 1,968,991 | Clickner          | Aug. 7, 1934  |
| 2,046,320 | Burbank           | July 7, 1936  |

## FOREIGN PATENTS

| Number  | Country       | Date          |
|---------|---------------|---------------|
| 467,812 | Great Britain | June 22, 1937 |
| 372,271 | Italy         | June 22, 1938 |
| 356,404 | France        | Nov. 29, 1905 |